

## UNITED STATES PATENT OFFICE

2,205,923

## PROCESS FOR CONCENTRATING ORES

Henry A. Doerner and Dwight L. Harris, Pullman,  
Wash., assignors to State College of Washington  
Research Foundation, Pullman, Wash.

No Drawing. Application January 9, 1939,  
Serial No. 249,895

8 Claims. (Cl. 209—167)

This invention relates to the process of concentrating ores by flotation. Flotation is accomplished chiefly by the action of reagents known as collectors. When such reagents are 5 added to a suspension of pulverized ore in water, they produce large complex ions that are selectively adsorbed by the various minerals. If the pulp is aerated, those mineral grains that have adsorbed the collecting ions become attached to 10 air bubbles, and are carried upward into a floating froth. In a flotation process the froth is skimmed off, thereby effecting a separation between the various minerals based upon the selective action of the collector. Other reagents may 15 be used to produce a better froth or to modify the selective action of the collector. These are called frothers, activators, depressors or conditioners.

Until recently, most, if not all collectors gave 20 negatively charge collecting ions. Such anionic collectors are strongly adsorbed by the metallic minerals, particularly the sulphides of heavy metals. In general they have relatively little effect on non-metallic minerals. Hence a separation 25 of metal sulphides from non-metallic minerals is easily accomplished. This selective action varies, and can be used to separate two or more easily floated minerals from each other. Such separations are more difficult and usually 30 require the assistance of activators or depressors to increase or reverse the selective action of the collector.

Recently, collectors of an opposite type have 35 been developed under trade names such as Emul-sol and D. P. Q. These give positive collecting ions that are adsorbed selectively by the non-metallic minerals. Although these cationic collectors have a much better selectivity with non-metallic minerals than the anionic reagents, the 40 degree of separation that can be obtained between most of the non-metallic minerals is far from complete.

We have found that if an ore containing several non-metallic minerals is first separated 45 into two or more products by flotation with one type of collector, and if one or more of those products are subsequently subjected to a second flotation with the opposite type of collector, the selective actions in the two steps are usually 50 cumulative. The separations thus made are more complete than can be accomplished by repeated flotation steps with only one type of collector. This is the essence of our invention.

We believe this discovery constitutes a new 55 principle in the art of flotation. It should not be confused with the common practice whereby the selectivity of a collector is modified or even reversed by the use of "addition agents." The changes in selectivity caused by "addition agents"

are usually cumulative when used first with one type and then with the other type of collector.

The principle can be illustrated by our process for the concentration of magnesite ores. Magnesite, as it occurs in nature, is commonly associated and more or less intimately mixed with dolomite, calcite, talc, serpentine and quartz. At present, magnesite of commercial grade is obtained by selective mining, hand sorting and washing. These methods are expensive, and can 10 not be used to obtain a high grade product from any but the best ores.

Several investigators have attempted to concentrate magnesite ores by flotation, but the results have not been good enough to encourage 15 commercial application. Two general methods have been tried; the flotation of impurities from the magnesite, and the flotation of magnesite from the impurities. The former gives best results with some ores, and with other ores the 20 latter method is more effective. But in general, neither method is adequate, and we have not found any claim that a separation has been made by flotation between the very similar minerals, magnesite and dolomite. 25

The cationic collectors are best for floating most of the siliceous material from magnesite ore. But in this case most of the dolomite and some silicates remain with the magnesite. Other investigators have shown that magnesite 30 can be floated with anionic collectors such as oleic acid. But in this case dolomite and some of the silicates also float and contaminate the product. The difficulty lies in the fact that in both cases some impurities float more readily 35 and others less readily than the magnesite. Nor is the selectivity sufficient to permit a clean separation by repeated flotation steps with the same type of collector.

We have found that if a siliceous product is 40 first removed by flotation with cationic collectors and then if magnesite is floated from the residual pulp by anionic collectors, a good recovery of the magnesite is obtained and the product is of much better grade than can be produced by previous methods. We have also found that the increased selectivity caused by certain conditioning reagents, such as tannin, is in this case also 45 cumulative.

For example, with cationic collectors, dolomite floats better than magnesite and the ratio of magnesite to dolomite is lower in the floated product than in the original material. When magnesite is subsequently floated with anionic collectors, it floats more readily than dolomite, 55 and thus the two separating effects are cumulative. The selectivity in each step, however, is so weak that even the cumulative separation is poor. But tannic acid, for example, will cause an increased selectivity in both steps and the 60

separation is then quite good. These steps also separate magnesite from other impurities even more completely than from dolomite.

The following table gives data that illustrate the foregoing discussion. The first line gives the analysis of the crude ore. About 30 percent of the MgO content of this ore is combined in the minerals, dolomite, serpentine and talc. Therefore a complete separation of the magnesite from all impurities will only give about 70 percent recovery of the total MgO. (See last column of the table.) When magnesite is heated to a high temperature it liberates CO<sub>2</sub> and is converted to MgO. The resulting calcine only weighs about half as much as the ore. The analyses in the table represent the composition of the calcined products.

In test #119 magnesite was floated with oleic acid. The ratio of MgO to CaO is slightly higher in this concentrate than in the crude ore.

In test #127 the pulp was conditioned with tannin and water glass, and then magnesite was floated with oleic acid. The ratio of MgO to CaO has been improved and the recovery is also higher.

In test #115 a siliceous product was floated with the cationic collector, "D. P. 243." In this case the "concentrate" is the material that failed to float. Although the ratio of MgO to CaO was only slightly improved, the grade and recovery are both better than was obtained in the previous tests.

#### Data from flotation tests

| No.                 | Percent of total weight | Percent volatile | Analysis of calcine percent |                                                                  |      |      | Percent of total MgO |
|---------------------|-------------------------|------------------|-----------------------------|------------------------------------------------------------------|------|------|----------------------|
|                     |                         |                  | SiO <sub>2</sub>            | Fe <sub>2</sub> O <sub>3</sub><br>Al <sub>2</sub> O <sub>3</sub> | CaO  | MgO  |                      |
| Ore.                |                         | 45.8             | 13.7                        | 2.3                                                              | 17.2 | 66.8 |                      |
| <i>Concentrates</i> |                         |                  |                             |                                                                  |      |      |                      |
| No.                 |                         |                  |                             |                                                                  |      |      |                      |
| 119                 | 64.8                    | 48.6             | 6.8                         | 2.1                                                              | 18.4 | 72.7 | 66.9                 |
| 127                 | 67.2                    | 47.9             | 9.2                         | 2.1                                                              | 12.9 | 75.8 | 70.0                 |
| 115                 | 70.1                    | 49.3             | 3.3                         | 2.1                                                              | 15.6 | 79.0 | 76.0                 |
| 147                 | 55.4                    | 50.3             | 2.4                         | 2.1                                                              | 11.4 | 84.1 | 70.0                 |
| 148                 | 44.0                    | 50.5             | 2.5                         | 2.0                                                              | 7.6  | 87.8 | 57.9                 |
| 149                 | 33.0                    | 50.7             | 2.6                         | 1.9                                                              | 5.8  | 80.7 | 45.8                 |
| 150                 | 43.5                    | 50.3             | 1.8                         | 2.1                                                              | 2.7  | 93.4 | 57.4                 |

In tests #147, #148, #149 and #150, the pulp was conditioned with tannin and a siliceous product was floated with D. P. 243. Then the enriched residue was conditioned with water glass and a magnesite concentrate floated with oleic acid. The ratio of MgO to CaO is 3.9 in the ore and 7.4, 11.5, 15.5 and 34.6 respectively in concentrates #147, #148, #149 and #150.

It is obvious that the order of the steps can be changed without departing from the spirit of the invention. For example, a concentrate floated by means of anionic collectors may be retreated by floating off impurities with cationic collectors. Nor do we limit our invention to the treatment of any particular kind of ore.

We claim:

1. The method of concentrating magnesite ore by flotation which comprises treating a water suspension of the comminuted ore in two steps: first, agitating and aerating the pulp with a cationic collector to produce and remove a froth containing chiefly siliceous impurities; second, agitating and aerating the remaining pulp with oleic acid to produce and remove a froth containing magnesite.

2. The method of concentrating magnesite ore by flotation which comprises treating a water

suspension of the comminuted ore in two steps: first, agitating and aerating the pulp with a cationic collector and a frothing agent to produce and remove a froth containing chiefly siliceous impurities; second, agitating and aerating the remaining pulp with oleic acid to produce and remove a froth containing magnesite.

3. The method of concentrating magnesite ore by flotation which comprises treating a water suspension of the comminuted ore in two steps: first, agitating and aerating the pulp with a cationic collector to produce and remove a froth containing chiefly siliceous impurities; second, agitating and aerating the remaining pulp with oleic acid to produce and remove a froth containing magnesite, plus the addition of sodium disilicate to increase the selectivity of the collector in one or both of the flotation steps.

4. The method of concentrating magnesite ore by flotation which comprises treating a water suspension of the comminuted ore in two steps: first, agitating and aerating the pulp with a cationic collector and a frothing agent to produce and remove a froth containing chiefly siliceous impurities; second, agitating and aerating the remaining pulp with oleic acid to produce and remove a froth containing magnesite, plus the addition of sodium disilicate to increase the selectivity of the collector in one or both of the flotation steps.

5. The method of concentrating magnesite ore by flotation which comprises treating a water suspension of the comminuted ore in two steps: first, agitating and aerating the pulp with a cationic collector to produce and remove a froth containing chiefly siliceous impurities; second, agitating and aerating the remaining pulp with oleic acid to produce and remove a froth containing magnesite, plus the addition of tannin to increase the selectivity of the collector in one or both of the flotation steps.

6. The method of concentrating magnesite ore by flotation which comprises treating a water suspension of the comminuted ore in two steps: first, agitating and aerating the pulp with a cationic collector and a frothing agent to produce and remove a froth containing chiefly siliceous impurities; second, agitating and aerating the remaining pulp with oleic acid to produce and remove a froth containing magnesite, plus the addition of tannin to increase the selectivity of the collector in one or both of the flotation steps.

7. The method of concentrating magnesite ore by flotation which comprises treating a water suspension of the comminuted ore in two steps: first, agitating and aerating the pulp with a cationic collector to produce and remove a froth containing chiefly siliceous impurities; second, agitating and aerating the remaining pulp with oleic acid to produce and remove a froth containing magnesite, plus the addition of a starch to increase the selectivity of the collector in one or both of the flotation steps.

8. The method of concentrating magnesite ore by flotation which comprises treating a water suspension of the comminuted ore in two steps: first, agitating and aerating the pulp with a cationic collector and a frothing agent to produce and remove a froth containing chiefly siliceous impurities; second, agitating and aerating the remaining pulp with oleic acid to produce and remove a froth containing magnesite, plus the use of a starch to increase the selectivity of the collector in one or both of the flotation steps.

HENRY A. DOERNER.  
DWIGHT L. HARRIS.